

# United States Patent [19]

El-Sayed

[11] Patent Number: 4,758,494

[45] Date of Patent: \* Jul. 19, 1988

[54] INORGANIC METAL SALT AS ADJUVANT FOR NEGATIVE LIQUID ELECTROSTATIC DEVELOPERS

[75] Inventor: Lyla M. El-Sayed, West Chester, Pa.

[73] Assignee: E. I. Du Pont de Nemours and Company, Wilmington, Del.

[\*] Notice: The portion of the term of this patent subsequent to Dec. 23, 2003 has been disclaimed.

[21] Appl. No.: 14,710

[22] Filed: Feb. 13, 1987

[51] Int. Cl.<sup>4</sup> ..... G03G 9/12

[52] U.S. Cl. ..... 430/137

[58] Field of Search ..... 430/115, 137

## [56] References Cited

### U.S. PATENT DOCUMENTS

3,779,926 12/1973 Merck et al. ..... 430/115

3,850,830 11/1974 Fukushima et al. ..... 430/115 X

3,959,153 5/1976 Sadamatsu et al. ..... 430/109 X

4,631,244 12/1986 Mitchell ..... 430/137

## FOREIGN PATENT DOCUMENTS

51-2828 1/1976 Japan ..... 430/115  
2169416A 7/1986 United Kingdom .

Primary Examiner—Roland E. Martin

## [57] ABSTRACT

Negative, liquid electrostatic developer consisting essentially of

- (A) nonpolar liquid having Kauri-butanol value less than 30, present in major amount,
- (B) thermoplastic resin particles having a colorant and an inorganic metal salt as defined dispersed therein and average particle size by area being less than 10  $\mu$ m, and
- (C) nonpolar liquid soluble ionic or zwitterionic compound which imparts a negative charge to the thermoplastic resin particles.

Optionally additional adjuvants are present. The liquid electrostatic developer is useful in copying, making proofs including digital color proofs, lithographic printing plates, and resists.

25 Claims, No Drawings

INORGANIC METAL SALT AS ADJUVANT FOR  
NEGATIVE LIQUID ELECTROSTATIC  
DEVELOPERS

DESCRIPTION

1. Technical Field

This invention relates to a negative-working liquid electrostatic developer having improved properties. More particularly this invention relates to a negative-working liquid electrostatic developer containing resin particles having dispersed therein an inorganic metal salt.

2. Background Art

It is known that a latent electrostatic image can be developed with toner particles dispersed in an insulating nonpolar liquid. Such dispersed materials are known as liquid toners or liquid developers. A latent electrostatic image may be produced by providing a photoconductive layer with a uniform electrostatic charge and subsequently discharging the electrostatic charge by exposing it to a modulated beam of radiant energy. Other methods are known for forming latent electrostatic images. For example, one method is providing a carrier with a dielectric surface and transferring a preformed electrostatic charge to the surface. Useful liquid toners comprise a thermoplastic resin and dispersant nonpolar liquid. Generally a suitable colorant is present such as a dye or pigment. The colored toner particles are dispersed in the nonpolar liquid which generally has a high-volume resistivity in excess of  $10^9$  ohm centimeters, a low dielectric constant below 3.0 and a high vapor pressure. The toner particles are less than  $10 \mu\text{m}$  average by area size. After the latent electrostatic image has been formed, the image is developed by the colored toner particles dispersed in said dispersant nonpolar liquid and the image may subsequently be transferred to a carrier sheet.

Since the formation of proper images depends on the differences of the charge between the liquid developer and the latent electrostatic image to be developed, it has been found desirable to add a charge director compound and preferably adjuvants, e.g., polyhydroxy compounds, aminoalcohols, polybutylene succinimide, an aromatic hydrocarbon, aluminum stearate, etc., to the liquid toner comprising the thermoplastic resin, dispersant nonpolar liquid, and preferably a colorant. Such liquid developers provide images of good resolution, but it has been found that charging and image quality are particularly pigment dependent. Some formulations, suffer from poor image quality manifested by significant low resolution, poor solid area coverage (density), and ghosting. In order to overcome such problems much research effort has been expended to develop new type charge directors and/or charging adjuvants for electrostatic liquid toners.

It has been found that the above disadvantages can be overcome and particularly improved ghosting properties achieved with developers prepared containing a dispersant nonpolar liquid, ionic or zwitterionic charge director compound, and a thermoplastic resin having a colorant, and having an inorganic metal salt dispersed in the resin.

DISCLOSURE OF THE INVENTION

In accordance with this invention there is provided an improved negative, liquid electrostatic developer consisting essentially of

(A) a nonpolar liquid having a Kauri-butanol value of less than 30, present in a major amount,

(B) thermoplastic resin particles having dispersed therein a colorant and an inorganic metal salt, wherein the cationic component of said inorganic metal salt is selected from the group consisting of the metals of Group Ia, Group IIa, and Group IIIa of the periodic table, and wherein the anionic component of said salt is selected from the group consisting of halogen, carbonate, acetate, sulfate, borate, nitrate, and phosphate, the resin particles having an average by areas particle size of less than  $10 \mu\text{m}$ , and

(C) a nonpolar liquid soluble ionic or zwitterionic charge director compound which imparts a negative charge to the thermoplastic resin particles.

In accordance with an embodiment of this invention there is provided a process for preparing a negative liquid electrostatic developer for electrostatic imaging containing thermoplastic toner particles comprising

(A) dispersing at an elevated temperature in a vessel a thermoplastic resin, a colorant, an inorganic metal salt, wherein the cationic component of said inorganic metal salt is selected from the group consisting of the metals of Group Ia, Group IIa, and Group IIIa of the periodic table, and wherein the anionic component of said salt is selected from the group consisting of halogen, carbonate, acetate, sulfate, borate, nitrate, and phosphate, a dispersant nonpolar liquid having a Kauri-butanol value of less than 30, and a colorant, while maintaining the temperature in the vessel at a temperature sufficient to plasticize and liquify the resin and below that at which the dispersant nonpolar liquid degrades and the resin and/or colorant decomposes,

(B) cooling the dispersion, either

(1) without stirring to form a gel or solid mass, followed by shredding the gel or solid mass and grinding by means of particulate media in the presence of additional liquid;

(2) with stirring to form a viscous mixture and grinding by means of particulate media in the presence of additional liquid; or

(3) while grinding by means of particulate media to prevent the formation of a gel or solid mass in the presence of additional liquid;

(C) separating the dispersion of thermoplastic toner particles having an average by area particle size of less than  $10 \mu\text{m}$  from the particulate media, and

(D) adding to the dispersion a nonpolar liquid soluble ionic or zwitterionic charge director compound which imparts a negative charge to the thermoplastic toner particles.

Throughout the specification the below-listed terms have the following meanings:

In the claims appended hereto "consisting essentially of" means the composition of the liquid electrostatic developer does not exclude unspecified components which do not prevent the advantages of the developer from being realized. For example, in addition to the primary components, there can be present additional components, such as fine particle size oxides, adjuvant, e.g., polyhydroxy compound, aminoalcohol, polybutylene succinimide, aromatic hydrocarbon, etc.

Aminoalcohol means that there is both an amino functionality and hydroxyl functionality in one compound.

Ghosting means there is developer in the background areas in the nontransferred or transferred image.

The dispersant nonpolar liquids (A) are, preferably, branched-chain aliphatic hydrocarbons and more particularly, Isopar®-G, Isopar®-H, Isopar®-K, Isopar®-L, Isopar®-M and Isopar®-V. These hydrocarbon liquids are narrow cuts of isoparaffinic hydrocarbon fractions with extremely high levels of purity. For example, the boiling range of Isopar®-G is between 157° C. and 176° C., Isopar®-H between 176° C. and 191° C., Isopar®-K between 177° C. and 197° C., Isopar®-L between 188° C. and 206° C. and Isopar®-M between 207° C. and 254° C. and Isopar®-V between 254.4° C. and 329.4° C. Isopar®-L has a mid-boiling point of approximately 194° C. Isopar®-M has a flash point of 80° C. and an auto-ignition temperature of 338° C. Stringent manufacturing specifications, such as sulphur, acids, carboxyl, and chlorides are limited to a few parts per million. They are substantially odorless, possessing only a very mild paraffinic odor. They have excellent odor stability and are all manufactured by the Exxon Corporation. High-purity normal paraffinic liquids, Norpar®12, Norpar®13 and Norpar®15, Exxon Corporation, may be used. These hydrocarbon liquids have the following flash points and auto-ignition temperatures:

| Liquid    | Flash Point (°C.) | Auto-Ignition Temp (°C.) |
|-----------|-------------------|--------------------------|
| Norpar®12 | 69                | 204                      |
| Norpar®13 | 93                | 210                      |
| Norpar®15 | 118               | 210                      |

All of the dispersant nonpolar liquids have an electrical volume resistivity in excess of 10<sup>9</sup> ohm centimeters and a dielectric constant below 3.0. The vapor pressures at 25° C. are less than 10 Torr. Isopar®-G has a flash point, determined by the tag closed cup method, of 40° C., Isopar®-H has a flash point of 53° C. determined by ASTM D 56. Isopar®-L and Isopar®-M have flash points of 61° C., and 80° C., respectively, determined by the same method. While these are the preferred dispersant nonpolar liquids, the essential characteristics of all suitable dispersant nonpolar liquids are the electrical volume resistivity and the dielectric constant. In addition, a feature of the dispersant nonpolar liquids is a low Kauri-butanol value less than 30, preferably in the vicinity of 27 or 28, determined by ASTM D 1133. The ratio of thermoplastic resin to dispersant nonpolar liquid is such that the combination of ingredients becomes fluid at the working temperature. The nonpolar liquid is present in an amount of 85 to 99.9% by weight, preferably 97 to 99.5% by weight, based on the total weight of liquid developer. The total weight of solids in the liquid developer is 0.1 to 15%, preferably 0.5 to 3.0% by weight. The total weight of solids in the liquid developer is solely based on the resin, including components dispersed therein, e.g., pigment component, adjuvant, etc.

Useful thermoplastic resins or polymers include: ethylene vinyl acetate (EVA) copolymers (Elvax®) resins, E. I. du Pont de Nemours and Company, Wilmington, DE), copolymers of ethylene and an  $\alpha,\beta$ -ethylenically unsaturated acid selected from the group consisting of acrylic acid and methacrylic acid, copolymers of ethyl-

ene (80 to 99.9%)/acrylic or methacrylic acid (20 to 0%)/alkyl (C<sub>1</sub> to C<sub>5</sub>) ester of methacrylic or acrylic acid (0 to 20%), polyethylene, polystyrene, isotactic polypropylene (crystalline), ethylene ethyl acrylate series sold under the trademark Bakelite® DPD 6169, DPDA 6182 Natural and DTDA 9169 Natural by Union Carbide Corp., Stamford, CN; ethylene vinyl acetate resins, e.g., DQDA 6479 Natural and DQDA 6832 Natural 7 also sold by Union Carbide Corp.; Surlyn® ionomer resin by E. I. du Pont de Nemours and Company, Wilmington, DE, etc., or blends thereof. Preferred copolymers are the copolymer of ethylene and an  $\alpha,\beta$ -ethylenically unsaturated acid of either acrylic acid or methacrylic acid. The synthesis of copolymers of this type are described in Rees U.S. Pat. No. 3,264,272, the disclosure of which is incorporated herein by reference. For the purposes of preparing the preferred copolymers, the reaction of the acid containing copolymer with the ionizable metal compound, as described in the Rees patent, is omitted. The ethylene constituent is present in about 80 to 99.9% by weight of the copolymer and the acid component in about 20 to 0.1% by weight of the copolymer. The acid numbers of the copolymers range from 1 to 120, preferably 54 to 90. Acid No. is milligrams potassium hydroxide required to neutralize 1 gram of polymer. The melt index (g/10 min) of 10 to 500 is determined by ASTM D 1238, Procedure A. Particularly preferred copolymers of this type have an acid number of 66 and 60 and a melt index of 100 and 500 determined at 190° C., respectively.

The thermoplastic resins described above have dispersed therein a pigment and an inorganic metal salt wherein the cationic component of the salt is selected from the group consisting of the metals of Group Ia, Group IIa, and Group IIIa, of the periodic table of elements (see CRC Handbook of Chemistry and Physics, 61st Edition, 1980-1981, Periodic Table of the Elements), and wherein the anionic component of said salt is selected from the group consisting of halogen, carbonate, acetate, sulfate, borate, nitrate, and phosphate. The cationic component metals include: sodium, potassium, barium, calcium, magnesium, strontium, aluminum, lithium, rubidium, cesium, and beryllium, etc. Examples of inorganic metal salts include: sodium chloride, sodium bromide, sodium acetate, potassium chloride, magnesium sulfate, calcium carbonate, cesium chloride, rubidium nitrate, beryllium sulfate, lithium bromide, rubidium acetate, strontium chloride, calcium acetate, aluminum sulfate, sodium borate, sodium phosphate, etc. The inorganic metal salt is present in 0.01 to 60 percent by weight, preferably 0.5 to 35 percent by weight based on the total weight of the developer solids. Particle size initially is preferably in the range of about 0.1 to 25  $\mu\text{m}$ . The method whereby the inorganic metal salt is dispersed in the thermoplastic resin is described below.

In addition, the resins have the following preferred characteristics:

1. Be able to disperse the inorganic metal salt, colorant, e.g., pigment,
2. Be insoluble in the dispersant liquid at temperatures below 40° C., so that the thermoplastic resin will not dissolve or solvate in storage,
3. Be able to solvate at temperatures above 50° C.,
4. Be able to be ground to form particles between 0.1  $\mu\text{m}$  and 5  $\mu\text{m}$ , in diameter,

5. Be able to form a particle (average by area) of less than 10  $\mu\text{m}$ , e.g., determined by Horiba CAPA-500 centrifugal automatic particle analyzer, manufactured by Horiba Instruments, Inc., Irvine, CA: solvent viscosity of 1.24 cps, solvent density of 0.76 g/cc, sample density of 1.32 using a centrifugal rotation of 1,000 rpm, a particle size range of 0.01 to less than 10  $\mu\text{m}$ , and a particle size cut of 1.0  $\mu\text{m}$ .

6. Be able to fuse at temperatures in excess of 70° C.

By solvation in 3. above, the resins forming the toner particles will become swollen or gelatinous.

Suitable nonpolar liquid soluble ionic or zwitterionic charge director compounds (C), which are generally used in an amount of 0.25 to 1500 mg/g, preferably 2.5 to 400 mg/g developer solids, include: negative charge 15 directors, e.g., lecithin, Basic Calcium Petronate®, Basic Barium Petronate® oil-soluble petroleum sulfonate, manufactured by Sonneborn Division of Witco Chemical Corp., New York, NY, etc.

As indicated above, colorants are dispersed in the 20 resin. Colorants, such as pigments or dyes and combinations thereof, the preferably present to render the latent image visible. The colorant, e.g., a pigment, may be present in the amount of up to about 60 percent by weight based on the total weight of developer solids, preferably 0.01 to 30% by weight based on the total weight of developer solids. The amount of colorant may vary depending on the use of the developer. Examples of pigments are Monastral® Blue G (C.I. Pigment Blue 15 C.I. No. 74160), Toluidine Red Y (C.I. Pigment Red 3), Quindo® Magenta (Pigment Red 122), Indo® Brilliant Scarlet (Pigment Red 123, C.I. No. 71145), Toluidine Red B (C.I. Pigment Red 3), Watchung® Red B (C.I. Pigment Red 48), Permanent Rubine F6B13-1731 (Pigment Red 184), Hansa® Yellow (Pigment Yellow 98), Dalamar® Yellow (Pigment Yellow 74, C.I. No. 11741), Toluidine Yellow G (C.I. Pigment Yellow 1), Monastral® Blue B (C.I. Pigment Blue 15), Monastral® Green B (C.I. Pigment Green 7), Pigment Scarlet (C.I. Pigment Red 60), Auric Brown (C.I. Pigment Brown 6), Monastral® Green G (Pigment Green 7), Carbon Black, Cabot Mogul L (black pigment C.I. No. 77266) and Sterling NS N 774 (Pigment Black 7, C.I. No. 77266).

Other ingredients may be added to the liquid electrostatic developer, such as fine particle size oxides, e.g., silica, alumina, titania, etc.; preferably in the order of 0.5  $\mu\text{m}$  or less can be dispersed into the liquefied resin. These oxides can be used in combination with the colorant. Metal particles can also be added.

Another additional component of the liquid electrostatic developer is an adjuvant which can be taken from the group of polyhydroxy compound which contains at least 2 hydroxy groups, aminoalcohol, polybutylene succinimide, metallic soap, and aromatic hydrocarbon having a Kauri-butanol value of greater than 30. The adjuvants are generally used in an amount of 1 to 1000 mg/g, preferably 1 to 200 mg/g developer solids. Examples of the various above-described adjuvants include:

polyhydroxy compounds: ethylene glycol, 2,4,7,9-tetramethyl-5-decyn-4,7-diol, poly(propylene glycol), pentaethylene glycol, tripropylene glycol, triethylene glycol, glycerol, pentaerythritol, glycerol-tri-12 hydroxystearate, ethylene glycol monohydroxystearate, propylene glycerol monohydroxystearate, etc.

aminoalcohol compounds: triisopropanolamine, triethanolamine, ethanolamine, 3-amino-1-propanol, o-

aminophenol, 5-amino-1-pentanol, tetra(2-hydroxyethyl)ethylenediamine, etc.

polybutylene succinimide: OLOA®-1200 sold by Chevron Corp., analysis information appears in Kosel U.S. Pat. No. 3,900,412, column 20, lines 5 to 13, incorporated herein by reference; Amoco 575 having a number average molecular weight of about 600 (vapor pressure osmometry) made by reacting maleic anhydride with polybutene to give an alkenylsuccinic anhydride which in turn is reacted with a polyamine. Amoco 575 is 40 to 45% surfactant, 36% aromatic hydrocarbon, and the remainder oil, etc.

metallic soap: aluminum tristearate; aluminum distearate; barium, calcium, lead and zinc stearates; cobalt, manganese, lead and zinc linoleates; aluminum, calcium, and cobalt octoates; calcium and cobalt oleates; zinc palmitate; calcium, cobalt, manganese, lead and zinc naphthenates; calcium, cobalt, manganese, lead and zinc resinate; etc. The metallic soap is dispersed in the thermoplastic resin as described in Trout, U.S. application Ser. No. 857,326, filed Apr. 30, 1986, the disclosure of which is incorporated herein by reference.

aromatic hydrocarbon: benzene, toluene, naphthalene, substituted benzene and naphthalene compounds, e.g., trimethylbenzene, xylene, dimethylethylbenzene, ethylmethylbenzene, propylbenzene, Aromatic 100 which is a mixture of C<sub>9</sub> and C<sub>10</sub> alkyl-substituted benzenes manufactured by Exxon Corp., etc.

The particles in the liquid electrostatic developer 30 have an average by area particle size of less than 10  $\mu\text{m}$ , preferably the average by area particle size is less than 5  $\mu\text{m}$ . The resin particles of the developer having the inorganic metal salt dispersed therein may or may not be formed having a plurality of fibers integrally extending therefrom although the formation of fibers extending from the toner particles is preferred. The term "fibers" as used herein means pigmented toner particles formed with fibers, tendrils, tentacles, threadlets, fibrils, ligaments, hairs, bristles, or the like.

The liquid electrostatic developer can be prepared by a variety of processes. For example, into a suitable mixing or blending vessel, e.g., attritor, heated ball mill, heated vibratory mill such as a Sweco Mill manufactured by Sweco Co., Los Angeles, CA, equipped with particulate media, for dispersing and grinding, Ross double planetary mixer manufactured by Charles Ross and Son, Hauppauge, NY, etc., or a two roll heated mill (no particulate media necessary) are placed at least one of thermoplastic resin, inorganic metal salt, and dispersant 50 nonpolar liquid described above. Generally the resin, colorant, metal salt, and dispersant nonpolar liquid are placed in the vessel prior to starting the dispersing step. Optionally the colorant can be added after homogenizing the resin and the dispersant nonpolar liquid. Polar additive can also be present in the vessel, e.g., up to 100% based on the weight of polar additive and dispersant nonpolar liquid. The dispersing step is generally accomplished at elevated temperature, i.e., the temperature of ingredients in the vessel being sufficient to plasticize and liquefy the resin but being below that at which the dispersant nonpolar liquid or polar additive, if present, degrades and the resin and/or colorant decomposes. A preferred temperature range is 80° to 120° C. Other temperatures outside this range may be suitable, however, depending on the particular ingredients used. The presence of the irregularly moving particulate media in the vessel is preferred to prepare the dispersion of toner particles. Other stirring means can

60

65

60

65

60

be used as well, however, to prepare dispersed toner particles of proper size, configuration and morphology. Useful particulate media are particulate materials, e.g., spherical, cylindrical, etc. taken from the class consisting of stainless steel, carbon steel, alumina, ceramic, zirconium, silica, and sillimanite. Carbon steel particulate media is particularly useful when colorants other than black are used. A typical diameter range for the particulate media is in the range of 0.04 to 0.5 inch (1.0 to approx. 13 mm).

After dispersing the ingredients in the vessel, with or without a polar additive present until the desired dispersion is achieved, typically 1 hour with the mixture being fluid, the dispersion is cooled, e.g., in the range of 0° C. to 50° C. Cooling may be accomplished, for example, in the same vessel, such as the attritor, while simultaneously grinding in the presence of additional liquid with particulate media to prevent the formation of a gel or solid mass; without stirring to form a gel or solid mass, followed by shredding the gel or solid mass and grinding, e.g., by means of particulate media in the presence of additional liquid; or with stirring to form a viscous mixture and grinding by means of particulate media in the presence of additional liquid. Additional liquid means dispersant nonpolar liquid, polar liquid or combinations thereof. Cooling is accomplished by means known to those skilled in the art and is not limited to cooling by circulating cold water or a cooling material through an external cooling jacket adjacent the dispersing apparatus or permitting the dispersion to cool to ambient temperature. The resin precipitates out of the dispersant during the cooling. Toner particles of average particle size (by area) of less than 10  $\mu\text{m}$ , as determined by a Horiba CAPA-500 centrifugal particle analyzer described above or other comparable apparatus, are formed by grinding for a relatively short period of time.

After cooling and separating the dispersion of toner particles from the particulate media, if present, by means known to those skilled in the art, it is possible to reduce the concentration of the toner particles in the dispersion, impart a negative electrostatic charge of predetermined polarity to the toner particles, or a combination of these variations. The concentration of the toner particles in the dispersion is reduced by the addition of additional dispersant nonpolar liquid as described previously above. The dilution is normally conducted to reduce the concentration of toner particles to between 0.1 to 10 percent by weight, preferably 0.3 to 3.0, and more preferably 0.5 to 2 weight percent with respect to the dispersant nonpolar liquid. One or more nonpolar liquid soluble ionic or zwitterionic charge director compounds (C), of the type set out above, can be added to impart a negative charge, as desired. The addition may occur at any time during the process; preferably at the end of the process, e.g., after the particulate media, if used, are removed and the concentration of toner particles is accomplished. If a diluting dispersant nonpolar liquid is also added, the ionic or zwitterionic compound can be added prior to, concurrently with, or subsequent thereto. If an adjuvant compound of a type described above has not been previously added in the preparation of the developer, it can be added prior to or subsequent to the developer being charged. Preferably the adjuvant compound is added after the dispersing step. It has been found that when the adjuvant is a polyhydroxy compound it is added after process step B or C.

Other process embodiments for preparing the liquid electrostatic developer include:

(A) dispersing a colorant and an inorganic metal salt as defined above in a thermoplastic resin in the absence of a dispersant nonpolar liquid having a Kauri-butanol value of less than 30 to form a solid mass.

(B) shredding the solid mass,

(C) grinding the shredded solid mass by means of particulate media in the presence of a liquid taken from 10 the group consisting of a polar liquid having a Kauri-butanol value of at least 30, a nonpolar liquid having a Kauri-butanol value of less than 30, and combinations thereof, thereby forming a dispersion of toner particles.

(D) separating the dispersion of toner particles having an average by area particle size of less than 10  $\mu\text{m}$  from the particulate media, and

(E) adding additional nonpolar liquid, polar liquid or combinations thereof to reduce the concentration of toner particles to between 0.1 to 15.0 percent by weight 20 with respect to the liquid; and

(F) adding to the dispersion a liquid soluble ionic or zwitterionic charge director compound which imparts a negative charge to the thermoplastic toner particles; and

(A) dispersing a colorant and an inorganic metal salt as defined above in a thermoplastic resin in the absence of a dispersant nonpolar liquid having a Kauri-butanol value of less than 30 to form a solid mass.

(B) shredding the solid mass,

(C) redispersing the shredded solid mass at an elevated temperature in a vessel in the presence of a dispersant nonpolar liquid having a Kauri-butanol value of less than 30, and optionally a colorant, while maintaining the temperature in the vessel at a temperature sufficient to plasticize and liquify the resin and below that at which the dispersant nonpolar liquid degrades and the resin and/or colorant decomposes,

(D) cooling the dispersion, and forming a dispersion of toner particles, either

(1) without stirring to form a gel or solid mass, followed by shredding the gel or solid mass and grinding by means of particulate media in the presence of additional liquid;

(2) with stirring to form a viscous mixture and grinding by means of particulate media in the presence of additional liquid; or

(3) while grinding by means of particulate media to prevent the formation of a gel or solid mass in the presence of additional liquid;

(E) separating the dispersion of toner particles having an average by area particle size of less than 10  $\mu\text{m}$  from the particulate media, and

(F) adding additional nonpolar liquid, polar liquid or combinations thereof to reduce the concentration of toner particles to between 0.1 to 15.0 percent by weight 55 with respect to the liquid; and

(G) adding to the dispersion a liquid soluble ionic or zwitterionic charge director compound which imparts a negative charge to the thermoplastic toner particles.

A preferred mode of the invention is described in Example 7.

#### INDUSTRIAL APPLICABILITY

The negative liquid electrostatic developers of this invention demonstrate improved image quality, solid area coverage (density), resolution and toning of fine details, evenness of toning, and particularly improved (reduced) ghosting independent of charge director and

pigment present. The particles are exclusively charged negative. The developers of this invention are useful in copying, e.g., making office copies of black and white as well as various colors; or color proofing, e.g., a reproduction of an image using the standard colors: yellow, cyan, magenta together with black as desired. In copying and proofing the toner particles are applied to a latent electrostatic image and can be transferred, if desired. Other uses are envisioned for the liquid electrostatic developers include: digital color proofing, lithographic printing plates, and resists.

### EXAMPLES

The following controls and examples wherein the parts and percentages are by weight illustrate but do not limit the invention. In the examples the melt indices were determined by ASTM D 1238, Procedure A; the average particle sizes by area were determined by a Horiba CAPA-500 centrifugal particle analyzer as described above, the density was measured using a Macbeth densitometer model RD918, transfer efficiency is determined as follows: a toned electrostatic image is transferred from the photoreceptor in the copier to a paper carrier sheet. A transparent adhesive tape is applied over the residual toned electrostatic image on the photoreceptor and the residual image is removed with the tape and placed on the previously image carrier sheet adjacent to (but not contacting) the transferred image. The density of both images is measured with a densitometer as previously described. The transfer efficiency is the percentage value obtained by dividing the density of the transferred image by the sum of the densities of the transferred and residual images. The resolution is expressed in the Examples in line pairs/mm (lp/mm). As noted in the examples and controls the following values for the indicated property are poor:

|                     |             |
|---------------------|-------------|
| Resolution          | below 5     |
| Density             | below 0.5   |
| Transfer Efficiency | below 65%   |
| Ghosting            | significant |

### EXAMPLE 1

In a Union Process 01 Attritor, Union Process Company, Akron, Ohio were placed the following ingredients:

| Ingredient                                                                                        | Amount (g) |
|---------------------------------------------------------------------------------------------------|------------|
| Copolymer of ethylene (89%) and methacrylic acid (11%) melt index at 190C is 100, Acid No. is 66. | 35.0       |
| Heuophthal Blue G XBT-583D                                                                        | 2.5        |
| Heubach, Inc., Newark, NJ                                                                         |            |
| Sodium Chloride, Aldrich Chemical Co., Milwaukee, WI                                              | 1.0        |
| Isopar ®-L, nonpolar liquid having a Kauri-butanol value of 27, Exxon Corporation                 | 125.0      |

The ingredients were heated to 100° C. ± 10° C. and milled at a rotor speed of 330 rpm with 0.1875 inch (4.76 mm) diameter stainless steel balls for two hours. The attritor was cooled to room temperature while the milling was continued, and then 125 grams of Isopar ®-H, nonpolar liquid having a Kauri-butanol value of 27, Exxon Corporation, were added. Milling was continued

at a rotor speed of 330 rpm for 22 hours to obtain toner particles with an average by area size of 1.49  $\mu\text{m}$ . The particulate media were removed and the dispersion of toner particles was then diluted to 1.0 percent solids with additional Isopar ®-H. To 1500 grams of the dispersion was added 20 milligrams of Lecithin (Aldrich Chemical Co.) in Isopar ®-H. Image quality was determined using a Savin 870 copier at standard mode: Charging corona set at 6.8 Kv and transfer corona set at 8.0 Kv using carrier sheets such as Plainwell off-set enamel paper number 3 class a 60 pound test. The results are shown below.

| Resolution | Density | Trans Eff. | Ghosting |
|------------|---------|------------|----------|
| 9.0        | 1.3     | 99%        | none     |

### EXAMPLE 2

A toner was prepared as described in Example 1 except that 3 grams of sodium bromide (Aldrich Chemical Co.) was used in place of sodium chloride. Milling was continued at a rotor speed of 330 rpm for 28 hours to obtain toner particles with an average by area size of 1.36  $\mu\text{m}$ . The particulate media were removed and the dispersion of toner particles was then diluted to 1.0 percent solids with additional Isopar ®-H. To 1500 grams of the dispersion was added 20 milligrams of Lecithin (Aldrich Chemical Co.) in Isopar ®-H. Image quality was determined as described in Example 1.

| Resolution | Density | Trans Eff. | Ghosting |
|------------|---------|------------|----------|
| 7.0        | 1.55    | 98%        | none     |

### EXAMPLE 3

A toner was prepared as described in Example 1 except that 1 g sodium acetate (Aldrich Chemical Co.) was used in place of sodium chloride. Milling was continued at a rotor speed of 330 rpm for 23.5 hours to obtain toner particles with an average by area size of 1.76  $\mu\text{m}$ . The particulate media were removed and the dispersion of toner particles was then diluted to 1.0 percent solids with additional Isopar ®-H. To 1500 grams of the dispersion was added 20.0 milligrams of Lecithin (Aldrich Chemical Co.) in Isopar ®-H. Image quality was determined as described in Example 1.

| Resolution | Density | Trans Eff. | Ghosting |
|------------|---------|------------|----------|
| 5.6        | 1.96    | 94%        | none     |

### EXAMPLE 4

A toner was prepared as described in Example 1 except that 3 g of potassium chloride (Aldrich Chemical Co.) were used in place of sodium chloride. Milling was continued at a rotor speed of 330 rpm for 15 hours to obtain toner particles with an average by area size of 0.93  $\mu\text{m}$ . The particulate media were removed and the dispersion of toner particles was then diluted to 1.0 percent solids with additional Isopar ®-H. To 1500 grams of the dispersion was added 20 milligrams of Lecithin (Aldrich Chemical Co.) in Isopar ®-H. Image quality was determined as described in Example 1.

| Resolution | Density | Trans Eff. | Ghosting |
|------------|---------|------------|----------|
| 8.0        | 1.53    | 97%        | none     |

## EXAMPLE 5

A toner was prepared as described in Example 1 except that 7 g magnesium sulfate (Aldrich Chemical Co.) was used in place of sodium chloride. Milling was continued at a rotor speed of 330 rpm for 22 hours to obtain toner particles with an average by area size of 1.61  $\mu\text{m}$ . The particulate media were removed and the dispersion of toner particles was then diluted to 1.0 percent solids with additional Isopar ®-H. To 1500 grams of the dispersion was added 16.6 milligrams of Lecithin (Aldrich Chemical Co.) in Isopar ®-H. Image quality was determined as described in Example 1.

| Resolution | Density | Trans Eff. | Ghosting    |
|------------|---------|------------|-------------|
| 9.0        | 1.4     | 98%        | reduced 90% |

## EXAMPLE 6

A toner was prepared as described in Example 1 except that 3 g calcium carbonate (Aldrich Chemical Co.) was used in place of sodium chloride. Milling was continued at a rotor speed of 330 rpm for 22 hours to obtain toner particles with an average by area size of 1.44  $\mu\text{m}$ . The particulate media were removed and the dispersion of toner particles was then diluted to 1.0 percent solids with additional Isopar ®-H. To 1500 grams of the dispersion was added 22 milligrams of Lecithin (Aldrich Chemical Co.) in Isopar ®-H. Image quality was determined as described in Example 1.

| Resolution | Density | Trans Eff. | Ghosting |
|------------|---------|------------|----------|
| 7.1        | 1.94    | 99%        | none     |

## EXAMPLE 7

A toner was prepared as in Example 1 except that 2 g of aluminum sulfate (Aldrich Chemical Co.) were used in place of sodium chloride. Milling was continued at a rotor speed of 330 rpm for 17 hours to obtain toner particles with an average by area size of 1.80  $\mu\text{m}$ . The particulate media were removed and the dispersion of toner particles was then diluted to 1.0 percent solids with additional Isopar ®-H. To 1500 grams of the dispersion was added 13.3 milligrams of Lecithin (Aldrich Chemical Co.) in Isopar ®-H. Image quality was determined as described in Example 1.

| Resolution | Density | Trans Eff. | Ghosting |
|------------|---------|------------|----------|
| 11.0       | 1.68    | 99%        | none     |

## EXAMPLE 8

A toner was prepared as described in Example 1 except that 3 g of sodium chloride were used. Milling was continued at a rotor speed of 330 rpm for 20.5 hours to obtain toner particles with an average by area size of 1.99  $\mu\text{m}$ . The particulate media were removed and the dispersion of toner particles was then diluted to 2.0 percent solids with additional Isopar ®-H. To 1500

grams of the dispersion was added 18.33 milligrams of Basic Barium Petronate ®, Aldrich Chemical Co. in Isopar ®-H. Image quality was determined as described in Example 1.

5

| Resolution | Density | Trans Eff. | Ghosting |
|------------|---------|------------|----------|
| 9.0        | 1.3     | 91%        | none     |

10

## EXAMPLE 9

A toner was prepared as in Example 1 except that 3 g of calcium acetate (Aldrich Chemical Co.) were used in place of sodium chloride. Milling was continued at a rotor speed of 330 rpm for 16 hours to obtain toner particles with an average by area size of 1.67  $\mu\text{m}$ . The particulate media was removed and the dispersion of toner particles was then diluted to 1.0 percent solids with additional Isopar ®-H. To 1500 grams of the dispersion was added 6.67 milligrams Basic Barium Petronate ®, Aldrich Chemical Co., in Isopar ®-H. Image quality was determined as described in Example 1.

15

| Resolution | Density | Trans Eff. | Ghosting |
|------------|---------|------------|----------|
| 9.0        | 0.48    | 83%        | none     |

20

## EXAMPLE 10

A toner was prepared as described in Example 1 except that 2 g of sodium borate (Aldrich Chemical Co.) were used in place of sodium chloride. Milling was continued at a rotor speed of 330 rpm for 19 hours to obtain toner particles with an average by area size of 1.44  $\mu\text{m}$ . The particulate media was removed and the dispersion of toner particles was then diluted to 1.0 percent solids with additional Isopar ®-H. To 1500 grams of the dispersion was added 6.67 milligrams of Lecithin, Aldrich Chemical Co., in Isopar ®-H. Image quality was determined as described in Example 1.

25

| Resolution | Density | Trans Eff. | Ghosting |
|------------|---------|------------|----------|
| 9.0        | 0.2     | 69%        | none     |

30

## EXAMPLE 11

A toner was prepared as described in Example 1 except that 1.59 g of sodium phosphate, dibasic anhydrous (Aldrich Chemical Co.) were used in place of sodium chloride. Milling was continued at a rotor speed of 330 rpm for 22.5 hours to obtain toner particles with an average by area size of 1.16  $\mu\text{m}$ . The particulate media was removed and the dispersion of toner particles was then diluted to 1.0 percent solids with additional Isopar ®-H. To 1500 g of the dispersion was added 22.2 milligrams of Basic Barium Petronate ® per gram toner solids in Isopar ®-H. Image quality was determined as described in Example 1.

35

| Resolution | Density | Trans Eff. | Ghosting |
|------------|---------|------------|----------|
| 7.1        | 0.83    | 82%        | none     |

40

## CONTROL 1

A toner was prepared as described in Example 1 except no sodium chloride was added. Milling was continued at a rotor speed of 330 rpm for 21 hours to obtain toner particles with an average by area size of 1.51  $\mu\text{m}$ . The particulate media were removed and the dispersion of toner particles was then diluted to 2.0 percent solids with additional Isopar ®-H. Image quality was determined as described in Example 1. Toner did not tone the charged areas of a selenium photoconductor covered drum but did tone the background areas via dielectrophoresis.

## CONTROL 2

A toner was prepared as described in Control 1 except that for Sample A, 5.5 milligrams Basic Barium Petronate ®, Aldrich Chemical Co., in Isopar ®-H were added to the 2 percent dispersion instead of the Lecithin used in Control 1 and for Sample B, 24 milligrams Basic Barium Petronate ®, Aldrich Chemical Co., in Isopar ®-H were added instead of the lecithin. Image quality was determined as described in Example 1.

| Sample | Resolution | Density | Trans Eff. | Ghosting |
|--------|------------|---------|------------|----------|
| A      | 5.6        | 0.30    | 31%        | none     |
| B      | 1.1        | 0.05    | 5%         | none     |

While this control shows improved ghosting, properties such as resolution, density and, in particular transfer efficiency are poor.

## CONTROL 3

A toner was prepared as described in Example 1 except no sodium chloride was added. Milling was continued at a rotor speed of 330 rpm for 17 hours to obtain toner particles with an average by area size of 1.60  $\mu\text{m}$ . The particulate media were removed and the dispersion of toner particles was then diluted to 2.0 percent solids with additional Isopar ®-H. To Sample A, 6.7 milligrams of Lecithin in Isopar ®-H were added. To sample B, 20 milligrams of Lecithin in Isopar ®-H were added. Image quality was determined as described in Example 1.

| Sample | Resolution | Density | Trans Eff. | Ghosting    |
|--------|------------|---------|------------|-------------|
| A      | 9.0        | 0.38    | 78%        | significant |
| B      | 6.3        | 0.48    | 95%        | significant |

What is claimed is:

1. A process for preparing negative, liquid electrostatic developer for electrostatic imaging comprising  
(A) dispersing at an elevated temperature in a vessel a thermoplastic resin, a colorant, an inorganic metal salt wherein the cationic component of said inorganic metal salt is selected from the group consisting of the metals of Group Ia, Group IIa, and Group IIIa of the periodic table, and wherein the anionic component of said salt is selected from the group consisting of halogen, carbonate, acetate, sulfate, borate, nitrate, and phosphate, a dispersant nonpolar liquid having a Kauri-butanol value of less than 30, while maintaining the temperature in the vessel at a temperature sufficient to plasticize and liquify the resin and below that at which the

dispersant nonpolar liquid degrades and the resin and/or colorant decomposes,

(B) cooling the dispersion, either

(1) without stirring to form a gel or solid mass, followed by shredding the gel or solid mass and grinding by means of particulate media in the presence of additional liquid;

(2) with stirring to form a viscous mixture and grinding by means of particulate media in the presence of additional liquid; or

(3) while grinding by means of particulate media to prevent the formation of a gel or solid mass in the presence of additional liquid;

(C) separating the dispersion of thermoplastic toner particles having an average by area particle size of less than 10  $\mu\text{m}$  from the particulate media, and

(D) adding to the dispersion a nonpolar liquid soluble ionic or zwitterionic compound which imparts a negative charge to the thermoplastic toner particles.

2. A process according to claim 1 wherein the cationic component is a metal selected from the group consisting of sodium, potassium, barium, calcium, magnesium, strontium, aluminum, lithium, rubidium, cesium, and beryllium.

3. A process according to claim 1 wherein the inorganic metal salt is a compound selected from the group consisting of sodium chloride, sodium bromide, sodium acetate, potassium chloride, magnesium sulfate, calcium carbonate, cesium chloride, rubidium nitrate, beryllium sulfate, lithium bromide, rubidium acetate, strontium chloride, calcium acetate, aluminum sulfate, sodium borate, and sodium phosphate.

4. A process according to claim 1 wherein there is present in the vessel up to 100% by weight of a polar additive having a Kauri-butanol value of at least 30, the percentage based on the total weight of the liquid in the developer.

5. A process according to claim 1 wherein the particulate media are selected from the group consisting of stainless steel, carbon steel, ceramic, alumina, zirconium, silica and sillimanite.

6. A process according to claim 1 wherein the thermoplastic resin is a copolymer of ethylene and an  $\alpha,\beta$ -ethylenically unsaturated acid selected from the group consisting of acrylic acid and methacrylic acid.

7. A process according to claim 1 wherein the thermoplastic resin is a copolymer of ethylene (80 to 99.9%)/acrylic or methacrylic acid (20 to 0%)/alkyl ester of acrylic or methacrylic acid wherein alkyl is 1 to 5 carbon atoms (0 to 20%).

8. A process according to claim 7 wherein the thermoplastic resin is a copolymer of ethylene (89%) methacrylic acid (11%) having a melt index at 190 ° C. of 100.

9. A process according to claim 1 wherein the ionic or zwitterionic compound is Basic Barium Petronate.

10. A process according to claim 1 wherein the ionic or zwitterionic compound is lecithin.

11. A process according to claim 1 wherein the additional dispersant nonpolar liquid polar liquid or combinations thereof is present to reduce the concentration of toner particles to between 0.1 to 15 percent by weight with respect to the liquid.

12. A process according to claim 11 wherein the concentration of toner particles is reduced by additional dispersant nonpolar liquid.

13. A process according to claim 1 wherein cooling the dispersion is accomplished while grinding by means of particulate media to prevent the formation of a gel or solid mass in the presence of additional liquid.

14. A process according to claim 1 wherein cooling the dispersion is accomplished without stirring to form a gel or solid mass, followed by shredding the gel or solid mass and grinding by means of particulate media in the presence of additional liquid.

15. A process according to claim 1 wherein cooling the dispersion is accomplished with stirring to form a viscous mixture and grinding by means of particulate media in the presence of additional liquid.

16. A process according to claim 1 wherein an adjuvant compound selected from the group consisting of 15 aminoalcohol, polybutylene succinimide, metallic soap, and an aromatic hydrocarbon is added during the dispersing step (A).

17. A process according to claim 16 wherein the adjuvant compound is an aminoalcohol.

18. A process according to claim 17 wherein the aminoalcohol is triisopropanolamine.

19. A process according to claim 11 wherein an adjuvant compound selected from the group consisting of 25 polyhydroxy compound, aminoalcohol, polybutylene succinimide, and an aromatic hydrocarbon is added to the liquid developer.

20. A process according to claim 19 wherein the adjuvant compound is a polyhydroxy compound.

21. A process according to claim 20 wherein the 30 polyhydroxy compound is ethylene glycol.

22. A process according to claim 19 wherein the adjuvant compound is a metallic soap.

23. A process according to claim 22 wherein the metallic soap is aluminum tristearate.

24. A process for preparing a negative liquid electrostatic developer comprising

(A) dispersing a colorant, an inorganic metal salt, wherein the cationic component of said inorganic metal salt is selected from the group consisting of 40 the metals of Group Ia, Group IIa, and Group IIIa of the periodic table, and wherein the anionic component of said salt is selected from the group consisting of halogen, carbonate, acetate, sulfate, borate, nitrate, and phosphate, in a thermoplastic resin in the absence of a dispersant nonpolar liquid having a Kauri-butanol value of less than 30 to 45 form a solid mass,

(B) shredding the solid mass,

(C) grinding the shredded solid mass by means of 50 particulate media in the presence of a liquid selected from the group consisting of a polar liquid having a Kauri-butanol value of at least 30, a non-polar liquid having a Kauri-butanol value of less than 30, and combinations thereof, thereby forming 55 a dispersion of toner particles,

(D) separating the dispersion of toner particles having an average by area particle size of less than 10  $\mu\text{m}$  from the particulate media, and

(E) adding additional nonpolar liquid, polar liquid or combinations thereof to reduce the concentration of toner particles to between 0.1 to 15.0 percent by weight with respect to the liquid; and

(F) adding to the dispersion a liquid soluble ionic or zwitterionic compound which imparts a negative charge to the thermoplastic toner particles.

25. A process for preparing a negative, electrostatic liquid developer comprising

(A) dispersing a colorant, an inorganic metal salt, wherein the cationic component of said inorganic metal salt is selected from the group consisting of the metals of Group Ia, Group IIa, and Group IIIa of the periodic table, and wherein the anionic component of said salt is selected from the group consisting of halogen, carbonate, acetate, sulfate, borate, nitrate, and phosphate, in a thermoplastic resin in the absence of a dispersant nonpolar liquid having a Kauri-butanol value of less than 30 to form a solid mass,

(B) shredding the solid mass,

(C) redispersing the shredded solid mass at an elevated temperature in a vessel in the presence of a dispersant nonpolar liquid having a Kauri-butanol value of less than 30, and optionally a colorant, while maintaining the temperature in the vessel at a temperature sufficient to plasticize and liquify the resin and below that at which the dispersant nonpolar liquid degrades and the resin and/or colorant decomposes,

(D) cooling the dispersion, and forming a dispersion of toner particles, either

(1) without stirring to form a gel or solid mass, followed by shredding the gel or solid mass and grinding by means of particulate media in the presence of additional liquid;

(2) with stirring to form a viscous mixture and grinding by means of particulate media in the presence of additional liquid; or

(3) while grinding by means of particulate media to prevent the formation of a gel or solid mass in the presence of additional liquid;

(E) separating the dispersion of toner particles having an average by area particle size of less than 10  $\mu\text{m}$  from the particulate media, and

(F) adding additional nonpolar liquid, polar liquid or combinations thereof to reduce the concentration of toner particles to between 0.1 to 15.0 percent by weight with respect to the liquid; and

(G) adding to the dispersion a liquid soluble ionic or zwitterionic compound which imparts a negative charge to the thermoplastic toner particles.

\* \* \* \* \*